# EUROPEAN PATENT SPECIFICATION

(11) **EP 0 395 359 B1**
(45) Date of publication and mention of the grant of the patent: **22.09.1993**
(21) Application number: 90304402.2
(22) Date of filing: 24.04.1990
(51) Int. Cl.: C10M 171/00

(54) **Electroviscous electrically insulating fluids**
Elektroisolierende elektroviskose Flüssigkeiten
Fluides électrovisqueux électriquement isolants

(30) Priority: 26.04.1989 JP 106997/89
(43) Date of publication of application: 31.10.1990
(73) Proprietor: Tonen Corporation, Tokyo 100 (JP)
(72) Inventor: Tomizawa, Hirotaka, c/o Tonen Corp., Res. and Dev., Iruma-gun, Saitama 354 (JP); Kanbara, Makoto, c/o Tonen Corp., Res. and Dev., Iruma-gun, Saitama 354 (JP); Hayafune, Masahiko, c/o Tonen Corp., Res. and Dev., Iruma-gun, Saitama 354 (JP)
(74) Representative: Diamond, Bryan Clive

(56) References cited:
- US-A- 2 751 352
- US-A- 3 047 507
- US-A- 3 367 872
- CHEMICAL ABSTRACTS, vol. 92, no. 2, 19th May 1980, page 127, abstract no. 166046u, Columbus, Ohio, US; S.D. LIKHTEROV et al.: "Electroviscous effect in oils containing additives", & KHIM. TEKHNOL. TOPL. MASEL 1980, (1), 43-5

## Description

The present invention relates to an electroviscous fluid, the viscosity of which can be controlled by applying voltage, and in particular to an electroviscous fluid, in which the viscosity is changed rapidly and reversibly from low temperature range to high temperature range when voltage is applied and a long and stable electroviscous effect is obtained and which can be used for electrical control of mechanical devices such as a clutch, valve or shock absorber.

An electro-rheological fluid or electroviscous fluid, in which the viscosity of the fluid is changeable by the application of voltage, has been known for many years (Duff, A.W., Physical Review, Vol. 4, No. 1 (1896) 23). Early studies on electroviscous fluids were concentrated on the system containing liquid only, and the effect was not strong enough. Later, studies have been made on the electroviscous fluid of a solid disperse system, where a considerable electroviscous effect could be obtained.

For example, Winslow proposed an electroviscous fluid, using paraffin, silica gel powder and adding water to make the system slightly electroconductive (Winslow, W.M., J. of Applied Physics, Vol. 20 (1949) 1137). From this study by Winslow, the electroviscous (electro-rheological) effect of the electroviscous fluid is called the ER effect or Winslow effect.

On the other hand, study has also been made of the mechanism of the electroviscous effect (ER effect) in the electroviscous fluid. For example, Klass reported that each particle, i.e. the dispersed phase in an electroviscous fluid, generates the induced polarization of the double layer in an electrical field and this was the primary cause of such effect (Klass, D.L. et al., J. of Applied Physics, Vol. 38, No. 1 (1967) 67). If this is explained from the principle of the electric double layer, the ions absorbed on the dispersed solids (such as silica gel) are evenly arranged on the outer surface of dispersed solids when E (electrical field) = 0, while polarization occurs in the ion distribution when E (electrical field) = finite value and each particle exerts an electrostatic action on each other in the electric field. Thus, each particle forms a bridge (cross-linkage) between electrodes and the shear-resistant force to the external stress, i.e., ER effect.

With full consideration given on the mechanism of the ER effect in the electroviscous fluid of this solid dispersing system, various proposals have been made to increase and to stabilize the viscosity of an electroviscous fluid. For example, a proposal was made to use silicon dioxide type fine particles, on which ferroelectric powder and a small quantity of water are absorbed (Japanese Provisional Patent Publication 53-17585), whereas this is disadvantageous and unsatisfactory in various points such as the response, the reproducibility of ER effect, low electroviscous effect, and the stability of ER effect for a long time. Particularly, the conventional electroviscous fluid containing moisture is disadvantageous in that water is evaporated at high temperature of more than 80°C. Further, even at less than 80°C, there are also problems such as instability due to the migration of moisture on the surface of the particles, the problem of durability by elution of electrode metal (such as copper) when high electric field is applied, the enhancement of ionization by increase in temperature and increase of electric current, or unstable temperature property, and other problems caused by the presence of moisture.

It is an object of this invention to provide an electroviscous fluid, by which it is possible to maintain the ER effect stably up to a high temperature of 100°C and to achieve high durability.

According to the present invention we provide an electroviscous fluid having an electrically insulating fluid as a dispersion medium, and in which is dispersed by weight:
(a) 0.1 to 50% of porous solid particles having a particle size of 10 nm to 200 µm;
(b) a polyhydric alcohol in an amount of 1 to 30% of the porous solid particles; and
(c) an antioxidant in an amount of 0.01 to 10% and/or a corrosion inhibitor in an amount of 0.001 to 10%, and
(d) at least one type of substance selected from an acid, salt or base in an amount of 0.01 to 5 wt%.

When a polyhydric alcohol and an acid, salt or base is added to the electroviscous fluid containing electrically insulating fluid and porous solid particles, the electroviscous effect is stabilized in a wide temperature range up to high temperature, and a high electroviscous effect is obtained. However, there is a problem as to durability because of the oxidation of electrically insulating fluid, porous solid particles or polyhydric alcohol, or the increase of electrically conductive substance caused by the corrosion of electrode under high voltage.

In the present invention, an antioxidant and/or corrosion inhibitor are added to such electroviscous fluid to obtain better effects in the responsiveness of viscosity change in a wide temperature range up to high temperature, reproducibility, electroviscous effect and, especially, durability.

Description is now given of each component of the electroviscous fluid according to the present invention.

First, as the electrically insulating fluid, which is the dispersion medium in the electroviscous fluid, a mineral oil or synthetic lubricant oil can for example be used. More specifically, there are oils such as a paraffinic oil, naphthenic oil, poly-α-olefin, polyalkylene glycol, silicone oil, diester, polyolester, phosphoric acid ester, silicon compound, fluorine compound or polyphenylether. An electroviscous fluid having a viscosity of 5 - 300 cP at 40°C can be used.

As the porous solid particles, for example, silica gel, moisture-containing resin, diatomaceous earth, alumina, silica-alumina, zeolite, an ion exchange resin or cellulose, can be used. The porous solid particles having a particle size of 10 nm - 200 µm are used in the ratio of 0.1 - 50 wt%. If it is less than 0.1 wt%. the ER effect is too low, and if it exceeds 50 wt%, the dispersing property is decreased.

A dispersing agent may optionally be used in the electroviscous fluid of this invention in order to disperse the porous solid particles evenly and stably.

Suitable dispersing agents are sulphonates, phenates, phosphonates, succinimide, amines or non-ionic dispersing agents, e. g., magnesium sulphonate, calcium sulphonate, calcium phosphonate, polybutenyl succinic acid imide, sorbitan mono-oleate or sorbitan sesqui -oleate. These are normally used at the ratio of 0.1 - 10 wt%, while they need not be used if the porous solid particles are easily dispersed.

As the polyhydric alcohol, dihydric alcohols and trihydric alcohols are effective. It is preferable to use ethylene glycol, glycerin, propanediol, butanediol or hexanediol; these substances are used at a ratio of 1 - 30 wt% of the porous solid particles, preferably at 2 - 15 wt%. If the ratio is less than 1 wt%, the ER effect is too low, and if it exceeds 30 wt%, this is undesirable because electric current then flows too easily.

Acid, salt or base components are included to obtain a higher ER effect. Polyhydric alcohol components keep the ER effect at a high temperature, while acid, salt or base components can increase the polarization effect. By using these components simultaneously, it is possible to increase the ER effect at high temperature.

As acid components, inorganic acids such as sulfuric acid, hydrochloric acid, nitric acid, perchloric acid, chromic acid, phosphoric acid or boric acid, or inorganic acids such as acetic acid, formic acid, propionic acid, lactic acid, isolactic acid, valeric acid, oxalic acid or malonic acid can be used.

As the salts, any compound consisting of a metal or base radical (such as NH₄⁺, N₂H₅⁺) and acid radical can be used. In particular, it is preferable to use a substance which dissolves in a polyhydric alcohol or mixture of polyhydric alcohol and water and is dissociated, or typical ionic crystal such as a halogenated compound of an alkali metal or alkali earth metal, or the alkali salt of an organic acid; e.g., LiCl, NaCl, KCl, MgCl₂, CaCl₂, BaCl₂, LiBr, NaBr, KBr, MgBr₂, LiI, NaI, KI, AgNO₃, Ca(NO₃)₂, NaNO₂, NH₄NO₃, K₂SO₄, Na₂SO₄, NaHSO₄, (NH₄)₂SO₄ or an alkali salt of an acid such as formic acid, acetic acid, oxalic acid or succinic acid.

A base to be used can be a hydroxide of an alkali earth metal, carbonate of an alkali metal or amine . It is preferable to use a substance which is dissolved in polyhydric alcohol or in the mixture of polyhydric alcohol and water and is disassociated, e.g., NaOH, KOH, Ca(OH)₂, Na₂CO₃, NaHCO₃, K₃PO₄, Na₃PO₄, aniline, an alkylamine or ethanolamine. The salt and the base as described above may be used simultaneously.

The acid, salt or base is be used in the ratio of 0.01 - 5 wt% to the entire electroviscous fluid. If it is less than 0.01 wt%, the ER effect is too low; and if it exceeds 5 wt%, it is not desirable because electric current flows more easily and the electric power consumption increase.

An essential component of the fluid is an antioxidant and/or corrosion inhibitor.

Antioxidant is added to prevent the oxidation of the electrically insulating liquid and polyhydric alcohol and also to stop the increase of electric conductivity due to the formation of oxidation products. Corrosion inhibitor is added to prevent the increase of electrical conductivity caused by the generation of metallic ions due-to the corrosion of the electrode (such as copper) under high voltage.

Antioxidants which are inactive to a polarizing agent and to the porous solid particles may be used, such as phenol-type or amine-type antioxidants. Suitable phenol-type antioxidants are 2,6-di-t-butyl-para-cresol, 4,4'-methylene-bis(2,6-di-t-butyl-phenol) and 2,6-di-t-butyl-phenol, suitable amine-type antioxidants are dioctyl-diphenyl-amine, phenyl-α-naphthyl-amine, an alkyl diphenyl amine or N-nitro-diphenyl amine. Preferably, 2,6-di-t-butyl-para-cresol or dioctyl-diphenyl-amine is used. These substances are used in the ratio of 0.01 - 10 wt% to the entire electroviscous fluid, and preferably 0.1 - 2.0 wt%. If the ratio is less than 0.01 wt%, the antioxidant effect is too low, and if it exceeds 10 wt%, problems occurs such as color tone deterioration, increased turbidity, generation of sludge and increase of viscosity.

It is preferable to use a corrosion inhibitor which is inactive to the polarizing agent and porous solid particles, e.g., nitrogen compounds such as benzotriazole and its derivatives, imidazoline, pyrimidine derivatives, and compounds containing sulfur and nitrogen, such as 1,3,4-thiadiazolepolysulfide, a 1,3,4-thiadiazolil-2,5-bis-dialkyl-dithiocarbomate, a 2-(alkyldithio)-benzoimidazole, β-(o-carboxybenzylthio)propionitrile or propionic acid; more preferably, benzotriazole or its derivatives are used. These substances are used in the ratio of 0.001 - 10 wt% to the entire electroviscous fluid, and preferably 0.01 - 1.0 wt%. If the ratio is less than 0.001 wt% there is no corrosion inhibition effect, and if it exceeds 10 wt%, problems occur such as color tone deterioration, increased turbidity, generation of sludge, and increase in the viscosity of the fluid.

The invention is now illustrated by the following examples and comparative example.

### Preparation of electroviscous fluid

- Mineral oil: 89.1% by wt
- silica gel: 6% by wt
- Ethylene glycol: 0.4% by wt
- Acetic acid (glacial): 0.5% by wt
- Succinimide: 4% by wt

The above substances are mixed together to make a basic fluid.

Using this basic mixture, various types of electroviscous fluids of the invention having the compositions given in Table 1 below were prepared: the ratios are by weight

The viscosity of the mineral oil was adjusted in such manner that all of these samples have a viscosity of 80 cP at 40°C.

In the above table, 2,6-di-t-butylphenol was used as the antioxidant (A) and dioctyldiphenylamine was used as (B). A benzotriazole derivative was used as the corrosion inhibitor (a) and imidazole was used as corrosion inhibitor (b).

The properties of the samples of the fluid were tested as follows:

With the above electroviscous fluids at 40°C and 90°C, the following parameters were measured using a voltage-applicable rotation viscosimeter:
- Responsiveness:
   Evaluated by the time (second) until viscosity is stabilized when AC electric field is changed from 0 to 2 x 10⁶ (V/m).
- Reproducibility:
   Evaluated by the ratio of viscosity change at the electric field of 2 x 10⁶ (V/m) when AC electric field is repeatedly changed in a cycle of 1 - 2 x 10⁶ (V/m) → 0.
- Durability:
   Evaluated by the variation (%) of the viscosity over time when AC electric field is stabilized at 2 x 10⁶ (V/m). (Measuring time: 5 hours)
- Electroviscous effect:
   Evaluated by the ratio of the viscosity at a AC electric field of 2 x 10⁶ (V/m) to the viscosity at an electric field of 0 (V/m).

The results of the evaluation are summarized in Table 2.

As is evident from Table 2, when an antioxidant and/or corrosion inhibitor is added to the electroviscous fluid, excellent effects are obtained, such as responsiveness of viscosity change in wide temperature range up to high temperature, reproducibility, electroviscous effect and durability.

## Claims

1. An electroviscous fluid having an electrically insulating fluid as a dispersion medium, and in which is dispersed by weight:
(a) 0.1 to 50% of porous solid particles having a particle size of 10 nm to 200 µm;
(b) a polyhydric alcohol in an amount of 1 to 30% of the porous solid particles;
(c) an antioxidant in an amount of 0.01 to 10% and/or a corrosion inhibitor in an amount of 0.001 to 10%; and
(d) at least one type of substance selected from an acid, salt or base in an amount of 0.01 to 5 wt%.

2. An electroviscous fluid according to Claim 1, wherein said antioxidant is of a phenol-type or an amine-type.

3. An electroviscous fluid according to Claim 1, wherein said antioxidant is 2,6-di-t-butyl-para-cresol, 4,4'-methylene-bis(2,6-di-t-butyl-phenol), 2,6-di-t-butyl phenol,dioctyl-diphenyl-amine, phenyl-α-naphthyl-amine, an alkyl diphenyl amine or N-nitro-diphenyl amine.

4. An electroviscous fluid according to Claim 1, wherein said antioxidant is benzotriazole or a derivative thereof, imidazoline, a pyrimidine derivative or a compound containing sulfur and nitrogen.

5. An electroviscous fluid as claimed in any preceding claim, which also includes an agent which assist the dispersion of the solid particles, in an amount of 0.1 to 10%.

6. An electroviscous fluid as claimed in Claim 5, wherein said agent is a sulphonate, phenate, phosphonate, succinimide, amine or non-ionic dispersing agent.

7. An electroviscous fluid as claimed in any preceding claim, wherein the electrically insulating fluid is a paraffinic oil, naphthenic oil, poly-α-olefin, polyalkylene glycol, silicon oil, diester, polyolester, phosphoric acid ester, silicon compound, fluorine compound or polyphenylether.

## Patentansprüche

1. Elektroviskose Flüssigkeit mit einer elektroisolierenden Flüssigkeit als einem Dispersionsmedium, in welchem nach Gewicht dispergiert ist:
a) 0,1 bis 50% poröser Festkörperpartikel mit einer Partikelgröße von 10nm bis 200µm;
b) ein mehrere Hydroxylgruppen enthaltender Alkohol in einer Menge von 1 bis 30% der porösen Festkörperpartikel;
c) ein Antioxidationsmittel in einer Menge von 0,01 bis 10% und/oder ein Korrosionsinhibitor in einer Menge von 0,001 bis 10%; und
d) wenigstens eine Art von Substanz ausgewählt aus einer Säure, Salz oder Base in einer Menge von 0,01 bis 5 Gew.-%.

2. Elektroviskose Flüssigkeit nach Anspruch 1, worin das Antioxidationsmittel von einer Phenolart oder einer Aminart ist.

3. Elektroviskose Flüssigkeit nach Anspruch 1, worin das Antioxidationsmittel 2,6-Di-t-Butyl-Para-Kresol, 4,4'-Methylen-Bis (2,6-Di-t-Butyl-Phenol), 2,6-Di-t-Butyl-Phenol, Dioctyl-Diphenyl-Amin, Phenyl-α-Naphthyl-Amin, ein Alkyldiphenylamin oder N-Nitro-Diphenylamin ist.

4. Elektroviskose Flüssigkeit nach Anspruch 1, worin das Oxidationsmittel Benzotriazol oder ein Derivat davon, Imidazolin, ein Pyrimidinderivat oder eine Schwefel oder Stickstoff enthaltende Verbindung ist.

5. Elektroviskose Flüssigkeit nach einem der vorangehenden Ansprüche, welche ebenso ein Mittel, welches die Dispersion der Festkörperpartikel unterstützt, in einer Menge von 0,1 bis 10% beinhaltet.

6. Elektroviskose Flüssigkeit nach Anspruch 5, worin das Mittel ein Sulfonat, Phenat, Phosphonat, Succinimid, Amin oder nichtionisches Dispersionsmittel ist.

7. Elektroviskose Flüssigkeit nach einem der vorangehenden Ansprüche, worin die elektroisolierende Flüssigkeit ein paraffinisches Öl, naphthenisches Öl, Poly-α-Olefin, Polyalkylenglykol, Silikonöl, Diester, Polyolester, Phosphorsäureester, Siliziumverbindung, Fluor-verbindung oder Polyphenyläther ist.

## Revendications

1. Fluide électrovisqueux ayant comme milieu de dispersion un fluide électriquement isolant, et dans lequel sont dispersés, en poids :
(a) 0,1 à 50 % de particules solides poreuses ayant une taille de 10 nm à 200 µm,
(b) un polyol dans une proportion de 1 à 30 % de ces particules solides poreuses,
(c) un antioxydant dans une proportion de 0,01 à 10 % et/ou un inhibiteur de corrosion dans une proportion de 0,001 à 10 %, et
(d) au moins un type de substance choisi parmi acide, base et sel, dans une proportion de 0,01 à 5 %.

2. Fluide électrovisqueux selon la revendication 1, dans lequel l'antioxydant est du type phénol ou du type amine.

3. Fluide électrovisqueux selon la revendication 1, dans lequel l'antioxydant est le di-tert-butyl-2,6 p-crésol, le méthylène bis-(di-tert-butyl-2,6 phénol)-4,4', le di-tert-butyl-2,6 phénol, la dioctyldiphénylamine, la phényl-α-naphtylamine, une alkyldiphénylamine ou la N-nitro-diphénylamine.

4. Fluide électrovisqueux selon la revendication 1, dans lequel l'antioxydant est le benzotriazole ou un dérivé de celui-ci, l'imidazoline, un dérivé de la pyrimidine ou un composé contenant du soufre et de l'azote.

5. Fluide électrovisqueux selon l'une des revendications précédentes, qui contient aussi, dans une proportion de 0,1 à 10 %, un agent aidant à la dispersion des particules solides.

6. Fluide électrovisqueux selon la revendication 5, dans lequel ledit agent est un sulfonate, un phénate, un phosphonate, le succinimide, une amine ou un agent dispersant non ionique.

7. Fluide électrovisqueux selon l'une des revendications précédentes, dans lequel le fluide électriquement isolant est une huile paraffinique, une huile naphténique, une poly-α-oléfine, un polyalcèneglycol, une huile silicone, un diester, un polyolester, un phosphate, un composé de silicium, un composé de fluor ou un polyphényléther.
